

July 23, 1929.

I. A. SHULIMSON

1,721,886

ELECTROLYTIC CELL

Filed Sept. 20, 1926

Fig. 1.



Fig. 2.



INVENTOR  
Israel A. Shulimson  
BY  
Evan A. Reuventhal  
ATTORNEY

## UNITED STATES PATENT OFFICE.

ISRAEL A. SHULIMSON, OF SPRINGFIELD, MASSACHUSETTS, ASSIGNOR TO AMERICAN BOSCH MAGNETO CORPORATION, OF SPRINGFIELD, MASSACHUSETTS, A CORPORATION OF NEW YORK.

## ELECTROLYTIC CELL.

Application filed September 20, 1926. Serial No. 136,400.

The present invention relates to electrolytic cells for alternating current rectifiers, electrolytic condensers, lightning arresters, and for other purposes, and has particular reference to the chemical composition of the cathodes and the electrolytes and the anodes of such cells, and to various combinations thereof in such cells, adapted especially for comparatively high voltages and low currents as in "B" battery eliminators for radio circuits or as a part of "A", "B" and "C" battery eliminators therefor.

It is well known that aluminum rectifies alternating currents in many solutions the most usual of which have been solutions of phosphates, fluorides, oxalates, tartrates, lactates, carbonates and borates, and, in general, salts of acids with complex anions and of weak organic acids. These solutions were mostly decidedly acidic, and corroded the electrodes markedly; and the reaction products consist largely of insoluble materials that precipitate and thus remove essential ingredients from the electrolytes, all of which impairs the life of the electrodes, unduly increases the internal resistance and temperature of the cell, and often prevents prompt starting, or even short circuits, the transformer or circuit supplying the current to the rectifier.

I found with an aluminum cathode, that a neutral solution of monobasic ammonium phosphate gives a fair degree of rectification and substantially no corrosion. Furthermore, this monobasic salt is the most stable of substantially all the phosphates, which highly recommends its use. Upon adding the chromate or dichromate of potassium or ammonium, the electrolyte becomes acidic and causes corrosion but the degree of the rectification and the voltage output are increased. Furthermore the chromate or dichromate stabilizes the rectifying film and decreases the internal resistance of the cell.

I also found upon neutralizing this solution, and in fact any of the above noted solutions and also solutions of chromates or dichromates of organic acids or acids with complex anions, or combinations thereof, that the corrosion is obviated, as a practical matter, at both electrodes, and that the degree of rectification and the voltage output are still further increased. Besides durion, which is extremely brittle and practically unmachinable, a steel or steel alloy or cast iron or lead

anode may be used in this electrolyte, and besides pure aluminum or an aluminum alloy such as duraluminum or magnalium may be used as the cathode. So also containers of steel or iron or lead may be used.

Furthermore, I found that a neutral solution of these various salts and combinations thereof may be obtained in various ways. Monobasic phosphate is acidic; dibasic phosphate is alkaline; a mixture can therefore form a neutral solution. Also dichromate is acidic, and with dibasic ammonium phosphate can form a neutral solution. If it is desired to further increase the number of acidic ingredients, as with oxalic, lactic, tartric or other acid, the excesses can still be brought back to neutrality with ammonium carbonate. The difficulties of titration may be overcome by using the ammonium carbonate for neutralization, applying as an indicator the noticeable cessation of the evolution of carbon-dioxide gas upon attaining neutrality. Even if an excess quantity of ammonium carbonate is used, no harmful effect occurs, since ammonium carbonate is itself a fair rectifying electrolyte with aluminum and its alloys.

Furthermore, I found that the addition of such ingredients as lactic acid, or glycerine or invert sugar, or combinations thereof, give desirable properties due to their colloidal characteristics. For example, glycerine supports a good deal of potential precipitation in a colloid form, which renders it unobjectionable, and it is itself reduced and oxidized in the process of electrolysis. Thus, if for any reason the electrolyte should tend toward acidity or basicity, a compensating oxidation or reduction of the glycerine tends to restore the equilibrium.

In all of the cells, one cathode and one anode may be employed for half wave rectification, or two cathodes and one anode may be employed for full wave rectification. Also the container may form the anode or act conjointly with an electrode for that purpose if made of the metals above noted.

For a "B" battery eliminator, I prefer to use an aluminum cathode, a chrome nickel steel anode and a steel container, with an electrolyte consisting by weight of about 15 per cent monobasic ammonium phosphate, 0.3 per cent potassium dichromate, 6 per cent ammonium carbonate and 1.25 per cent glycerine, in water. For an electrolytic con-

denser, I prefer to reduce the proportions of monobasic ammonium phosphate, the potassium dichromate and the ammonium carbonate to about 2 per cent, 0.2 per cent and 0.8 per cent, respectively.

In the accompanying drawing illustrating the preferred form of my invention in application, as an example, to a full wave rectifier for a "B" battery eliminator for radio receiving sets, Fig. 1 is a sectional elevation of the cell; and Fig. 2 is a diagram of the electrical circuits. Each of the cells has a container 1 of steel with a perforated cover 2 of insulating material through which extend 10 an aluminum rectifying cathode 3 and an anode 4 of chrome nickel steel. The electrolyte 5 consists of 300 ccm. of water, 60 grams of monobasic ammonium phosphate, 12 grams of potassium dichromate, 24 grams of ammonium carbonate for neutralizing the solution, and 4 ccm. of glycerine (approximately 5 grams). A layer of oil 6 is floated upon the electrolyte to reduce evaporation. The cathode 3 has a rounded end at 7 to prevent erosion from bubble streams during electrolysis and has most of its length covered with a hard rubber sleeve 8 screwed against a shoulder as shown to present about 2.5 sq. cm. of rectifying surface each and to prevent disintegration 25 of the cathodes at the place where the surface of the electrolyte may be at the time.

As shown in Fig. 2, the four cells 9 are arranged in a bridge with the terminals of the secondary 10 of a transformer connected to 30 two opposite points thereof and a suitable filter circuit, containing inductances 11 and condensers 12, connected to the two other opposite points thereof. The primary 13 of the transformer is connected to an alternating 40 current circuit 14, 15, and the other terminals 16, 17 of the filter circuit are connected to the plate circuit of the receiving set (not shown). Usually the circuit 14, 15 is of about 120 volts, in which case the transformer ratio is about 45 1 to 1.3 to impress about 150 volts on the bridge.

These electrolytic cells deliver about 30 milliamperes at about 150 volts for several thousands of hours. The rectifying films on 50 the cathodes remain imperforate and adherent, and likewise the protective film on the anodes. The cells start into operation almost instantly. The temperature rise of each cell is only 5° C. from ordinary room 55 temperature, after an output from the bridge of 30 milliamperes for 8 hours. The efficiency of rectification is about 90 per cent at 30 milliamperes output from the bridge.

I claim—

60 1. In an electrolytic cell, a cathode com-

prising aluminum, an anode, and an electrolyte containing a neutralized solution of a phosphate of ammonium and a chromate of potassium.

2. In an electrolytic cell, a cathode comprising aluminum, an anode, and an electrolyte containing a neutralized solution of monobasic phosphate of ammonium and a chromate of potassium. 65

3. In an electrolytic cell, a cathode comprising aluminum, an anode, and an electrolyte containing a neutralized solution of monobasic phosphate of ammonium and potassium dichromate. 70

4. In an electrolytic cell, a cathode comprising aluminum, an anode, and an electrolyte containing a neutralized solution containing monobasic phosphate of ammonium 10 per cent to 20 per cent and potassium dichromate 0.1 per cent to 5 per cent. 75

80 5. In an electrolytic cell, a cathode comprising aluminum, an anode, and an electrolyte composed of a solution of monobasic phosphate of ammonium and a chromate of potassium rendered non-acidic with ammonium carbonate.

85 6. In an electrolytic cell, a cathode comprising aluminum, an anode, and an electrolyte composed of a solution of monobasic phosphate of ammonium and dichromate of potassium rendered non-acidic with ammonium carbonate. 90

95 7. In an electrolytic cell; an electrolyte containing a substantially neutralized solution of monobasic phosphate of ammonium and a chromate of potassium; a cathode containing aluminum mainly; and an anode containing iron mainly.

100 8. In an electrolytic cell; an electrolyte composed of a solution of monobasic phosphate of ammonium, a chromate of potassium, and ammonium carbonate sufficient to neutralize the solution; a cathode containing aluminum mainly; and an anode containing iron mainly.

105 9. In an electrolytic cell; an electrolyte composed of a solution of monobasic phosphate of ammonium, a chromate of potassium, glycerine, and ammonium carbonate sufficient to neutralize the solution; a cathode containing aluminum mainly; and an anode containing iron mainly. 110

115 10. In an electrolytic cell; an electrolyte composed of a solution of monobasic phosphate of ammonium, a chromate of potassium, glycerine, and ammonium carbonate sufficient to neutralize the solution; a cathode containing aluminum mainly; an anode containing iron mainly; and a steel container.

In testimony whereof I affix my signature

ISRAEL A. SHULIMSON.